

# UNITED STATES PATENT OFFICE

SAMUEL S. WALES, OF MUNHALL, PENNSYLVANIA, ASSIGNOR TO CARNEGIE STEEL COMPANY, OF PITTSBURGH, PENNSYLVANIA, A CORPORATION OF NEW JERSEY.

## ARMOR-PLATE.

1,111,709.

Specification of Letters Patent. Patented Sept. 22, 1914.

No Drawing.

Application filed August 1, 1906. Serial No. 328,659.

To all whom it may concern:

Be it known that I, SAMUEL S. WALES, of Munhall, in the county of Allegheny, State of Pennsylvania, have invented an Improvement in Armor-Plate, of which the following is a specification.

Of recent years it has been the practice in the manufacture of armor plate to make the plate of steel having substantially the following theoretical composition: carbon, .28 per cent.; manganese, .35 per cent.; nickel, 3.75 per cent.; chromium, 1.70 per cent., the sulfur and silicon being low,—below .04 per cent. The steel of this composition is then treated by the Harvey or Krupp processes by which its surface is highly supercarburized for the purpose of rendering it more resistant to the impact of projectiles. While the process of supercarburizing improves the surface it is detrimental in its effect upon the body of the plate.

I have discovered a new composition and a new process of treatment, by which I am enabled to make armor plate of homogeneous chemical composition without the necessity of supercarburizing the surface, and my plate will give much better results in resisting the impact of projectiles than have heretofore been obtained. For example, a six-inch plate which I have made according to my invention, has resisted the impact of a shell having a velocity 15 to 20 per cent. greater than that which could be resisted by the best Krupp plates of similar thickness. My invention is therefore of great importance, because it enables me to produce an armor plate having great tenacity and strength, of homogeneous composition, and capable of resisting shocks much better than any armor plate which heretofore has been produced.

The elements which I alloy with the iron in order to produce my new steel, are as follows, and in stating them I desire to premise that in addition to these elements, those skilled in the art may add other elements if desired, or may vary the proportions within certain limits, the proportions which I give being those which I have heretofore found best suited to the purpose: carbon, .15 to .25 per cent.; manganese, .15 to .35 per cent.; nickel, 5 to 12 per cent.; chromium, .15 to .25 per cent.; tungsten,

.50 to .70 per cent. To these elements I may add vanadium or molybdenum from .20 to .50 per cent., or I may substitute vanadium or molybdenum in place of tungsten in whole or in part.

The steel which I employ is open hearth steel, and I prefer to add the nickel as a part of the charge of the furnace in a cold condition and to add the manganese, chromium and tungsten in the ladle, or to add them in the furnace just before tapping, although the time and manner of addition may be varied. The proper proportion of carbon is had by recarburing in accordance with usual methods. The silicon content of the steel should be as low as possible, say, less than .15 per cent. The sulfur and phosphorus are respectively preferably less than .04 per cent.

The new heat treatment to which I subject the steel is covered in Patent No. 921,925, granted to me on May 18, 1909 for a Method of Treating Armor or Deck Plates, is as follows: Having cast the ingot and forged it at the ordinary forging temperature, if it is to be reforged it is subjected to a heat treatment in which it is raised to a temperature of about 700 degrees C., and cooled slowly, preferably in air. It may then be reforged at the usual reforging temperature, and is then heated to a temperature of about 875 degrees C., which is higher than that to which the plates are reheated in the Krupp process. It is then quenched with water, the duration of the water treatment being preferably about one minute per inch of thickness, the time varying according to the chemical composition of the steel, being preferably somewhat less when the carbon content is higher. If the steel is not reforged, the heating to 875 degrees C., and the quenching will immediately follow the forging; the plate not being allowed to become cold in the meantime. The steel is then raised to a temperature of about 775 degrees C., which is also higher than that to which the steel is raised at this period in the Krupp process, and it is then allowed to cool slowly, preferably in air, and may be rough-machined. If the plate needs forming it is then reheated, preferably to about 750 degrees C., at which temperature it may be bent or straightened as desired, the requisite being that the temperature shall be less than that

of the last preceding heat treatment. The plate is then annealed by being heated preferably to about 500 degrees C. by one or more successive treatments, and is allowed 5 to cool in air. It is then finally machined. The plate is then ready for the final water hardening, which may be conducted in any suitable way. I prefer, however, to accomplish this water-hardening by a new method, 10 in which I heat the entire body of the plate uniformly to a temperature of about 725 to 775 degrees C., and then quench it with water applied simultaneously on both surfaces so as to harden the plate uniformly through- 15 out its body. I then soften the plate on one surface by heating it on one side only, while the other surface is protected from the heat by loam or otherwise, the temperature being carried preferably to say 500 to 550 de- 20 grees C., the effect of which is to soften one surface of the plate, leaving the other side with substantially its original hardness. On removing it from the furnace I spray the harder surface of the plate in order to pre- 25 vent the equalization of the heat in the body of the plate and its softening throughout.

Those skilled in the art will be able to

modify the steps of the heat treatment above described within certain limits, since

What I claim is:

1. A steel armor plate containing silicon, manganese, nickel, chromium and tungsten; the nickel being in excess of 5 per cent, the chromium less than .25 per cent. and the tungsten less than .70 per cent.

2. A steel armor plate containing silicon, manganese, nickel, chromium and tungsten, the nickel being present in the proportion of from 5 to 12 per cent, the chromium in the proportion of from .15 to .25 per cent, and the tungsten in the proportion of from .50 to .70 per cent.

3. A steel armor plate containing silicon up to .15 per cent, not more than .35 per cent. manganese, at least 5 per cent. nickel, less than .25 per cent. chromium and less than .70 per cent. tungsten.

In testimony whereof, I have hereunto set my hand, July 28th, 1906.

SAMUEL S. WALES.

Witnesses:

THOMAS W. BAKENELL,  
W. R. BALSINGER.